

July 12, 1938.

J. HEILMANN

2,123,778

ELECTRIC WIRE

Filed March 22, 1935



Inventor:  
J. Heilmann,  
By G. F. Wunderoth  
Att'y.

## UNITED STATES PATENT OFFICE

2,123,778

## ELECTRIC WIRE

Josué Heilmann, Clichy, France, assignor to Société Alsacienne de Constructions Mécaniques, Clichy, France

Application March 22, 1935, Serial No. 12,497  
In France December 12, 1934

15 Claims. (Cl. 205—18)

Finished products in which the conducting core is insulated from the outer metallic sheathing by means of a solid pulverulent body have already been produced. In such processes a work-piece

5 having an initial size which will give the final size desired is subjected to drawing to produce a wire of a given diameter and length.

The manufacturing processes heretofore used failed to secure conducting or resistance wires of 10 high electrical properties and particularly failed in producing a perfectly homogeneous dielectric material having an exactly centered core (either with a single integral or stranded core or with a core comprising a plurality of conductors) and a 15 high kilometric insulating resistance.

The present invention has for its object a manufacturing process overcoming the above mentioned disadvantages and producing a product materially different from the products heretofore 20 manufactured.

The invention first of all comprises a complete dehydration of the dielectric to remove all water whether of composition, crystallization or suspension. The work piece is then preferably tightly 25 sealed before being subjected to the metallurgical treatments. In fact, the inventor has ascertained that complete dryness of the dielectric permits reaching insulating resistances of much higher range than those obtained with the same but 30 not completely dehydrated dielectric. Consequently a new type of electric wire is produced.

Such dehydration causes a new stability of the wire involving the new and very useful feature of high temperature resistance. This feature 35 means, first, that the electric wire can withstand, without any disadvantage, a high temperature at which the presence of vaporized water in ordinary wires entrapped in the compressed insulating material, which becomes impervious due to its considerable length, would involve the danger of explosion of the sheathing, and second that it is practically possible, without danger or any disadvantage to subject the wire to a temperature beyond which the metals constituting the sheathing 40 and the core are burnt or molten ordinarily. The new wire can withstand a temperature at which electric wires or cables heretofore manufactured would be destroyed.

Another feature of the invention consists in 45 arranging the dielectric within the metallic sheathing under a homogeneous, isotropic and compact form and to this end said dielectric is reduced to a fine powder and compressed under a proper pressure.

50 Such pressure is sufficiently high to secure a

compactness hereinafter called limit compactness so that external stresses applied to the sheathing are completely transmitted to the core through the dielectric.

In one example of the process, the insulation, 5 prior to its insertion in the sheathing, is shaped into compressed elements by moulding under high pressure. Such elements are then arranged by hand in the work-piece.

In another example, the insulation in the form 10 of a powder is directly compressed within the sheathing of the work-piece under suitable pressure.

The work-piece thus obtained is subsequently 15 subjected to metallurgical treatments comprising shrinking and drawing in several courses, to secure a very considerable length.

Electric conducting or resistance wires are secured comprising a continuous metallic sheathing, a single integral or stranded conductor or a 20 plurality of conductors and having an intermediate insulation such as magnesia or steatite, which is completely dehydrated, homogeneous and compact. The insulating resistance and thermal conductivity of such electric conductors are both very 25 high.

By way of example and in order to facilitate the 30 understanding of the invention, an example thereof will be hereafter described.

The apparatus intended to compress the insulation in pulverulent form will be described 35 with reference to the accompanying drawing in which:

Figure 1 is a longitudinal sectional view of a 40 work piece during the filling.

Figures 2 and 3 are respectively plan and elevational views of a tup-hammer for a single conductor work-piece.

Fig. 4 is a cross sectional view of the completed 45 wire.

The insulating material used is pulverulent magnesia but other materials such as steatite could as well be used.

The said insulating material, either in the form 50 of powder or of compressed elements of such powder, is subjected to a complete dehydration, which will be continued until the last traces of water, whether composition, crystallization or suspension, has disappeared. Practically, drying will be continued until after the weight of the material ceases to vary.

A thermal cycle which gives good results for magnesia consists in heating at 1112° F. for 3 hours.

In inserting the insulation in the sheathing, 55

care must be taken to avoid re-hydration. To this end the work-piece may be heated during such operation.

The finished work-piece is heated for some minutes in a high temperature kiln and the piece is preferably tightly closed in order to avoid any alteration during subsequent treatments.

The work-piece may be closed by means of asbestos washers and a metal washer secured there-  
10 to in any desired manner.

According to the invention, the insulation is inserted in the work-piece sheathing under such compactness or limit compactness that the external pressures applied to the sheathing are  
15 completely transmitted to the core and consequently it is not necessary to subject the work-piece to a shrinking treatment before being able to obtain a homothetic lengthening after drawing.

20 According to the materials being tested, the value of the pressure which gave the best results was 57,000 lbs. per square inch for magnesia and 14,200 lbs. per square inch for steatite.

The insulating material may be brought to the compact state in various ways, either in the form  
25 of compressed elements obtained under high pressure or by pressing it directly in the work-piece or in any other convenient way.

When the pulverulent insulation is introduced  
30 in the form of compressed elements, said elements are agglomerated by a press capable of exerting a pressure which corresponds to the above mentioned values. The blocks thus obtained are subsequently dehydrated and successively introduced within the work-piece.

35 When the pulverulent insulating material is to be directly compressed into the sheathing the device shown in the accompanying drawing may be used.

40 The sheath-tube of the work-piece T is ar- ranged vertically upon a bearing of convenient form and is provided at its lower part with a metallic washer forming a complete closure. The core passes through the washer and is firmly se- cured to the same.

45 In order that the insulating material may be rapidly compressed into the sheathing, the lower part of the tube should be clamped in a vise or like device E, in order to withstand all the stresses and particularly the tensile strength applied by  
50 a spring to the core for maintaining its recti- linear shape.

At the top of the sheath tube is arranged a funnel K in order to facilitate the flow of the insulating material.

55 Prior to securing the core to the spring R a tup-hammer M is inserted between the wire or wires of the core and the tube, said tup hammer being intended to compress the material. Its shape is determined for compressing the powder introduced between its surface and the tube and for centering the wires.

60 Good results have been obtained with the type shown in Figures 2 and 3. The tup hammer is fitted to the end of a tube D, which is of sufficient length so that the hammer may reach the lower end of the sheath-tube. In said position, the upper end of the tube D will sufficiently extend from the sheath tube so as to secure at O a machine (not shown) which operates the hammer in the  
70 manner of a pile driver.

The funnel K is supplied by a device (not shown) which is filled with pulverulent material treated as explained above. The tup hammer carrier tube is subjected to a positive ascending  
75 motion and then to a free fall or controlled mo-

tion. The magnesia falls between the front part of the tup hammer and the sheath-tube and is compressed. In the meanwhile the core is ex-  
actly centered and the level of the insulating ma-  
terial gradually rises in the work-piece. The  
5 ascending and falling motion of the hammer is combined with a rotating motion intended to pro-  
duce a uniform compacting. Further, in order to facilitate the operation of the tup hammer car-  
rier tube the latter may be made in several sec-  
tions connected by threaded sleeves.

The finished work-piece is then subjected to drawing in successive courses. Due to the prop-  
erties obtained by the above mentioned treat-  
ments, it will be possible to considerably increase  
15 the length of the electric wire, the respective di-  
mensions of sheathing, insulation and core re-  
maining homothetic.

The electric wires thus obtained distinguish  
20 from those heretofore produced by their struc-  
ture as well as by their properties. They are pro-  
vided with a completely dehydrated, highly com-  
pact dielectric constituted by grains of very small  
25 size, compressed under high pressure for attaining  
the limit compactness of the dielectric, and  
consequently very homogeneous and isotropic.

The kilometric insulating resistance of such  
electric wires is of a much higher range than those  
heretofore manufactured. Said resistance is  
30 much higher than 10 megohms and for a type of  
cable in which the internal diameter of the sheath  
tubing is  $1\frac{1}{4}$  in. and the core diameter  $\frac{1}{8}$  in.  
the resistance will be higher than 2000 megohms.

In a more general way, the resistivity of the  
insulation at 68° F. (for magnesia) is higher than  
35  $6 \times 10^6$  megohms per square centimeter section  
of insulation and per centimeter of length. For  
the above mentioned cable the resistivity reached  
12  $\times 10^8$  megohms per square centimeter and per  
centimeter.

40 Furthermore, the insulation has a very homo-  
geneous state and a very high degree of com-  
pactness or limit compactness giving for mag-  
nesia a density of about 2.3.

Finally the thermal conductivity of the insula-  
tion reaches and even goes beyond  $15\frac{1}{1000}$  watt per  
45 centimeter of length and per degree C. For the  
example given above the thermal conductivity  
was higher than  $25\frac{1}{1000}$  watt.

As a new industrial product, the invention also  
50 relates to the work-piece provided with agglomer-  
ated and dehydrated dielectric. The work-  
piece is preferably tightly closed at its ends in  
order to avoid any introduction of water during  
subsequent treatments.

55 The invention applies to the manufacture of  
wires or cables of all types, provided with one  
or more conductors whether for high or low cur-  
rents, high or low tension, energy transmission  
or heating purposes. The electric wires thus  
60 obtained are highly resistant to heat; their  
overall thermal conductivity is very high and  
consequently avoids the danger of burning due  
to overload; the insulation is practically inde-  
structible (the perforation of the insulation fol-  
65 lowing accidental excess voltage leaves the in-  
sulation practically untouched), and consequent-  
ly a high security is provided against excess  
voltages; the insulating resistance is very high  
70 and the dielectric features of such electric wires  
are absolutely stable.

According to the above mentioned process the  
wires may be made in sections of considerable  
length.

Having now particularly described and ascer-  
75

tained the nature of my invention and in what manner the same is to be performed, I declare that what I claim is:

1. A process of manufacturing fireproof electric wires comprising a conducting core, a refractory insulation and a metal sheath, by drawing an initial work-piece composed of such elements, characterized by the fact that before the said metallurgical drawing treatment, the insulation is subjected to a complete dehydration in order to eliminate all the water physically and chemically bound which is contained in the insulation, and preserved from all rehydration until the metallurgical treatments.
2. A process according to claim 1, in which the insulation is subjected to a complete dehydration by the elimination of all the water physically and chemically bound, which it contains and is then immediately inserted in the sheath of the work-piece whereupon said work-piece is subsequently subjected to the metallurgical drawing treatments.
3. A process of manufacturing fireproof electric wires comprising surrounding a conducting core located in a metallic sheath with refractory material, subjecting said refractory material to a complete dehydration in order to eliminate all water physically and chemically bound therein and then subjecting said core, sheath and refractory material to a metallurgical drawing treatment.
4. A process as set forth in claim 3 in which said refractory material is subjected to a complete dehydration for the elimination of all water physically and chemically bound prior to the insertion of said refractory material about said core.
5. A process as set forth in claim 3 in which said refractory material is subjected to a complete dehydration at the temperature of at least 600° C. for a period of about three hours prior to the insertion of said material about said core.
6. A process according to claim 1, in which before the metallurgical drawing treatment the insulation is subjected to a complete dehydration in order to eliminate all the water physically and chemically bound it contains and to a compression corresponding to the state of limit compactness of the said insulation.
7. A process as set forth in claim 3 in which said refractory material is subjected to high pressure when being disposed about said core.
8. A process as set forth in claim 3 in which said refractory material is essentially magnesium oxide and in which said magnesium oxide is subjected to a pressure above 4000 kg./cm<sup>2</sup>.
9. A process according to claim 1 in which the insulation is magnesium oxide and is subjected before the metallurgical drawing treatment to a complete dehydration in order to eliminate all the water physically and chemically bound which is contained in said insulation and to a compression above 4000 kg./cm<sup>2</sup>.
10. A process according to claim 3 in which said refractory material is essentially steatite and in which said steatite is subjected to a pressure in excess of 1000 kgs./cm<sup>2</sup>.
11. A process as set forth in claim 3 in which said refractory material is compressed in the form of moulded blocks under high pressure and in which said blocks are subjected to a complete dehydration in order to eliminate the water physically and chemically bound therein prior to their insertion about said conducting core within said sheath.
12. A process according to claim 1 in which the insulation is compressed in the form of blocks moulded under a pressure which is corresponding to the state of limit compactness of the insulation, the said blocks being subsequently subjected to a complete dehydration in order to eliminate the water physically and chemically bound, then inserted into the sheath of the work-piece, said work-piece being subsequently subjected to the metallurgical treatments in order to reduce its diameter to the required size.
13. A fire proof electric wire comprising an external metallic sheath, a conducting metallic core located within said sheath and parallel to the axis and a pulverulent insulation inserted between said sheath and said core, said insulation being under pressure and having a physically and chemically anhydrous state and the kilometric insulating resistance of said wire being in excess of 2000 megohms.
14. A fireproof electric wire comprising a continuous external metal sheath, a conducting metal core parallel to the axis and a pulverulent insulation inserted therebetween, said insulation being in the state of limit compactness, in a physically and chemically anhydrous state and the resistivity of the insulating being, at the ordinary temperature, higher than  $6 \times 10^8$  megohms per square centimeter section of insulation and per centimeter of length.
15. A process as set forth in claim 3 in which said refractory material is magnesium oxide and is subjected to a complete dehydration at a temperature of at least 600° C. for a period of about three hours prior to the insertion of said material about said core.

JOSUÉ HEILMANN.